

Aug. 1, 1961

W. A. GEY

2,994,597

SLOW BURNING PROPELLENT GRAIN WITH POLYSULFIDE POLYMER COATING

Filed Feb. 20, 1953



INVENTOR.  
WILLIAM A. GEY

## 1

2,994,597

SLOW BURNING PROPELLANT GRAIN WITH  
POLYSULFIDE POLYMER COATINGWilliam A. Gey, China Lake, Calif., assignor to the  
United States of America as represented by the Sec-  
retary of the Navy

Filed Feb. 20, 1953, Ser. No. 338,177

1 Claim. (Cl. 52—5)

(Granted under Title 35, U.S. Code (1952), sec. 266)

The invention described herein may be manufactured and used by or for the Government of the United States of America for governmental purposes without the payment of any royalties thereon or therefor.

This invention relates to slow burning propellant grain and the method of making it.

In most applications of propellents, such as rocketry, a propellant grain having a fast burning rate is desired. However, in some applications, such as the driving of servo-mechanisms and other similar devices, a slow burning propellant grain which gives a longer operation time for the device powered by it is required. Propellant grains ordinarily used to power high speed devices have too rapid a burning rate for use in servo-mechanisms. In addition, previous propellant grains are subject to the disadvantage that separations are formed in them under operating conditions because of the widely different coefficient of expansion of the compressed grain and the adjacent container wall. This results in irregular burning which causes excessive and widely varying pressures which are impossible to control, thus making the use of previous propellant grains highly impractical in such devices as servo-mechanisms which must be susceptible of precise control.

It is, therefore, an object of this invention to provide a slow burning propellant grain.

It is another object of this invention to provide a propellant grain for use in servo-mechanisms which can be packaged and used under operating conditions without the formation of separations due to different coefficients of expansion of the compressed grain and the adjacent container wall.

It has been found that the above objects can be accomplished and the enumerated difficulties overcome by a propellant grain coated with a restrictive coating of a cured polysulfide polymer.

The propellant used to illustrate this invention comprises a mixture of about 75 parts of nitroguanidine, 25 parts of guanidine nitrate, and 8 parts of ammonium dichromate. The nitroguanidine used is a high bulk density product. The guanidine nitrate is practical grade, ground to pass a 100-mesh screen. The ammonium dichromate is chemically pure, or practical and is ground to pass a 200-mesh screen.

The propellant grain in this case was formed by compressing the dry powder mixture in a 1.125" diameter polished steel mold at 27,000 pounds per square inch. In order to properly compact the powder, two pressings of 23 grams each are made. The ram for the first pressing contains a conical cavity in order to insure proper adhesion of the second increment. The ram for the second pressing is flat. After pressing, the burning surface was modified by cutting cross slots three thirty seconds inch wide into the face with a circular saw to a depth of nine-sixteenths inch. This cavity is required to obtain the desired burning area to nozzle area ratio of 1180 which yields an operating pressure of 1000 p.s.i. at ordinary temperatures. The larger initial burning area also compensates for the initial heat loss to the cold metal chamber.

The function of the restrictive coating or liner is to absorb the differential thermal expansion between grain

## 2

and container and maintain a tight fit against the grain. It must be strong and stiff with a surface hard and smooth enough to resist damage or slippage during loading of the fuel. Combined with these properties the coating of this invention has the property of restricting the burning surface of the propellant grain. The restrictive coating used is a liquid polysulfide polymer or poly-functional mercaptan, designated commercially as "Thiokol," LP-2, which has been cured. "Thiokol" LP-2 is made in accordance with the process set forth in U.S. Patent 2,466,963, granted April 12, 1949, to Joseph C. Patrick and Harry R. Ferguson. The polymer has the following properties:

## Properties

|    |                       |                |
|----|-----------------------|----------------|
| 15 | Molecular weight, av. | 4000.          |
|    | Viscosity, poises     | 350 to 450.    |
|    | pH                    | 6-8.           |
|    | Specific gravity      | 1.27.          |
| 20 | Color                 | Amber.         |
|    | Stability             | Indefinite.    |
|    | Moisture content      | Less than .2%. |

## Formula:



SH terminals—Extremely reactive.

The burning surface restrictant, Thiokol LP-2, was cured by mixing 100 parts of it with a previously mixed suspension of 9 parts of lead oxide, 8.5 parts of dibutyl phthalate, and 0.5 part of stearic acid, and warming at 50° C. for 16 hours. Chemically pure lead oxide, PbO<sub>2</sub>, must be used, as the mixture is sensitive to impurities and will "cure" rapidly in the cold in their presence.

35 The procedure for application of the restrictant consisted in painting the grain (except for the coned end) with a cold-curing, rubber-to-metal cement, for example, that designated by Navy specification No. 52-C-15 Type I, drying until tacky, placing it in a mold which had been

40 treated with silicone release agent, and pouring the uncured mixture of inhibitor around the grain. The curing operation was carried out under 4 to 5 inches of vacuum to remove air bubbles. A firm rubbery coating .060 inch thick was obtained. The inhibitor was found to 45 control the burning rate of the grain, the finished grain of a diameter of 1 1/8 inches burning at a rate of .14 inch per second at 1000 p.s.i. This burning rate is in contrast to that of prior propellants which have burning rates impossible to check. When tested in a servomotor the grain proved satisfactory.

50 The rubbery quality of the inhibitor coating removes the disadvantages formerly resulting from different coefficients of expansion of container and grain, i.e., separations of the grain. The inhibitor coating forms a 55 moisture-proof enclosure for the grain and enhances both its storage qualities and handling characteristics.

The drawing shows a typical pressure-time trace of the propellant grain illustrating its burning characteristics.

60 While there has been disclosed a preferred embodiment of my invention in which a specific propellant composition is used with the cured polysulfide restrictant, to illustrate the invention, the example is by no means intended to be limiting. It will be apparent to those skilled in the art that the weight proportions of the components in the propellant composition may be varied depending upon the burning rate required. Also, propellants of totally different composition may be used in combination with the burning surface restrictant.

65 70 It is thus seen that there has been disclosed a propellant grain adapted for use in servo-mechanisms and other mechanisms of this type which has a slow burning rate,

good handling and storage characteristics and which is easily fabricated.

Obviously many modifications and variations of the present invention are possible in the light of the above teaching. It is, therefore, to be understood that within the scope of the appended claims the invention may be practiced otherwise than as specifically described.

What is claimed is:

A propellant grain consisting essentially of about 75 parts by weight of nitroguanidine, about 25 parts by weight of guanidine nitrate, about 8 parts by weight of ammonium dichromate, and a coating on the outer surface of said grain consisting of a cured polysulfide polymer having the average structure



**References Cited in the file of this patent**

**UNITED STATES PATENTS**

|           |               |               |
|-----------|---------------|---------------|
| 2,195,380 | Patrick       | Mar. 26, 1940 |
| 2,479,828 | Geckler       | Aug. 23, 1949 |
| 2,555,333 | Grand et al.  | June 5, 1951  |
| 2,584,264 | Foulks        | Feb. 5, 1952  |
| 2,637,274 | Taylor et al. | May 5, 1953   |
| 2,643,184 | Cairns et al. | June 23, 1953 |

**OTHER REFERENCES**

Murray: "Aircraft Gas-Turbine Fuels," in The Oil and Gas Journal, March 29, 1951, page 279.

McLaren, Rocket Engine Fuels, in Automotive and Aviation Industries, August 15, 1946, page 22.

Thiokol, Liquid Polymer LP-2, Thiokol Chemical Corp., Trenton, N.J., revised January 20, 1949.